

2,980,518

## INHIBITING GEL FORMATION IN FUEL OILS

Philip L. Bartlett, Wilmington, Del., assignor to E. I. du Pont de Nemours and Company, Wilmington, Del., a corporation of Delaware

No Drawing. Filed Aug. 27, 1956, Ser. No. 606,186

20 Claims. (Cl. 44—66)

This invention relates to inhibiting the formation of copper mercaptide gels in hydrocarbon distillate fuel oils and to liquefying preformed copper mercaptide gels.

It is known that a gel frequently is formed in hydrocarbon distillate fuel oils under storage and service conditions, such as in domestic oil burner installations, diesel service and the like, and forms gelatinous deposits in the equipment which plug lines, orifices, filter screens, and the like. The gel is formed in the presence of copper or brass equipment, such as brass filters, floats and needle valves, and copper tubing and contains copper mercaptides which act as the gelling agents. This gel is conventionally known as copper mercaptide gel and is not soluble in conventional solvents. The formation and deposition of the gel presents a serious problem, as it has been necessary to strip down the systems and manually remove the gel therefrom.

It has been discovered that the copper mercaptide gels derive from active mercaptans present in the fuel oil and that they are readily produced under actual or simulated field conditions from hydrocarbon distillate fuels containing active mercaptans. These gels consist substantially of minor proportions of copper mercaptide (approximately 0.1 to 1.0%), the copper being in the cuprous form, and of major proportions of hydrocarbon components (at least 95% and sometimes over 99%); also small quantities of oxygenated material and water are often present. The usual fuel oil sludge inhibitors are ineffective in preventing formation of such gel and in breaking up existing gel.

Sulfur compounds generally occur as impurities in all petroleum hydrocarbon products, the type and quantity of the sulfur compounds being determined by the source and previous processing history of the petroleum product. Mercaptans, in particular, have hitherto been objectionable to the industry for various reasons (odor, corrosiveness, etc.) and many processes have been devised for converting them into innocuous materials or for eliminating them more or less completely from petroleum products. However, like all refining processes, these are costly, and some are rather inefficient in destroying or removing mercaptans. As a result, many hydrocarbon distillate fuels are often marketed unrefined or only partially refined, with mercaptans still present in various amounts, depending on their ultimate use, particularly fuel oils designated as burner, heating, or furnace oil. The mercaptan sulfur content of such fuel oils may range from as low as 0.001 weight percent to as high as about 0.03 weight percent.

Where careful refining of all grades of hydrocarbon distillates is economically impractical, it would be preferable to be able to provide an additive to prevent formation of copper mercaptide gel or, in the event gelation does occur, to break up the gel and thus unplug service equipment.

It is an object of this invention to provide hydrocarbon distillate fuel oils containing compounds which inhibit the formation of copper mercaptide gel therein and the depo-

sition of such gels on surfaces in contact therewith. Another object is to provide concentrated solutions of such inhibitors for ready and economical transportation and use thereof, including particularly for use in liquefying preformed copper mercaptide gel. A further object is to provide a process for liquefying copper mercaptide gel and, particularly, for removing deposits of such gel from equipment. Other objects are to provide new compositions of matter and to advance the art. Still other objects will appear hereinafter.

The above and other objects may be accomplished in accord with this invention which comprises (1) a hydrocarbon distillate fuel oil which contains at least one mercaptan which normally tends to form a copper mercaptide gel and to which fuel oil there has been added a small proportion, sufficient to inhibit such gel formation, of at least one polyamino compound of the group consisting of alkylene primary diamines of 2 to 10 carbon atoms in which the primary amino groups are separated by 2 to 6 carbon atoms, dialkylene triamines of 4 to 10 carbon atoms in which the amino groups are separated by 2 to 4 carbon atoms and two of the amino groups are primary amino groups, and mono-acid salts of said diamines and said triamines in which the acids are selected from the group consisting of monocarboxylic fatty acids of 8 to about 22 carbon atoms, monohydric mononuclear phenols, and monocarboxylic petroleum naphthenic acids of about 8 to about 29 carbon atoms; (2) the process of liquefying a gel, formed by the action of a copper mercaptide on a normally liquid hydrocarbon, by adding to said gel at least 1% by weight of at least one of said polyamino compounds, as such or as a concentrated solution in a normally liquid hydrocarbon; and (3) concentrated solutions of at least one of said polyamino compounds in a normally liquid hydrocarbon.

It has been found that the polyamino compounds of this invention, when added in a small proportion to a hydrocarbon distillate fuel oil that contains at least one mercaptan which normally tends to form a copper mercaptide gel when the fuel oil is brought into contact with copper or brass, are very effective to inhibit such gel formation and the deposition of such gel on surfaces with which the fuel oil may be brought into contact. It has been found further that when small proportions of said polyamino compounds, as such or as concentrated solutions in normally liquid hydrocarbons, are added to copper mercaptide gels, the gels are broken up (liquefied) and can be readily removed from equipment by washing with a normally liquid hydrocarbon, whereby such equipment can be unplugged and cleaned of such gels without stripping down or dismantling the equipment.

The alkylene primary diamines and the dialkylene triamines together may be represented by the formula:



where  $m$  is equal to 0 or 1, alkylene is a divalent saturated aliphatic hydrocarbon radical  $—\text{C}_n\text{H}_{2n}\text{—}$ , and the nitrogen atoms are bonded to different carbon atoms. In the alkylene primary diamines,  $m$  is equal to 0,  $n$  represents an integer of 2 to 10, preferably 2-6, and the two  $\text{NH}_2$  groups are separated by 2 to 6 carbon atoms, preferably 2 to 4 carbon atoms. In the dialkylene triamines,  $m$  is equal to 1,  $n$  in each alkylene group represents an integer of 2 to 8, preferably 2 to 4, and the number of carbon atoms in the two alkylene groups total 4 to 10, preferably 4 to 8, and the  $—\text{NH—}$  group is separated from each  $—\text{NH}_2$  group by 2 to 4 carbon atoms, preferably 2-3 carbon atoms. The alkylene groups may be straight or branched chain. The amino groups may be attached to primary, secondary or tertiary carbon atoms; the term "primary" in "alkylene primary diamine" referring to the primary amino groups ( $—\text{NH}_2$ ).

In the dialkylene triamines, the alkylene units may be the same or different. Homologous alkylene primary diamines and dialkylene triamines containing more than 10 carbon atoms, while operable, are generally less desirable for reasons of cost and economy.

Representative alkylene diamines are: ethylene diamine; 1,2-propylene diamine; 1,3-propylene diamine; 1,3-diamino-2-methylpropane, 1,3-diamino-2,2-dimethylpropane; the 1,2-, 1,3-, 1,4-, and 2,3-butylene diamines and carbon-alkylated derivatives such as 2,3-diamino-2-methylbutane and 1,4-diamino-2-ethylbutane; pentylene diamines typified by 1,2-, 2,4-, and 1,5-diaminopentane, including carbon alkylated compounds such as 1,4-diamino-4-methylpentane and 2,4-diamino-2,4-dimethylpentane; hexylene diamines represented by 1,6-hexylene diamine (hexamethylene diamine) and 2,4-hexylene diamine, and including higher homologs such as 2,5-diamino-2,5-dimethylhexane.

Typical dialkylene triamines of this invention are: 1,2-diethylene triamine; 1,2- and 1,3-dipropylene triamine; and the corresponding dibutylene triamines in which each pair of nitrogen atoms in the chain is separated by at least 2 carbon atoms.

Fuel oil soluble mono-acid salts of the hereinbefore defined alkylene primary diamines and dialkylene triamines are also effective for the purposes of this invention. Such mono-acid salts contain one mole of the acid for each mole of the polyamine and are prepared by methods well known and conventional in the art, such as by mixing the polyamine with the organic acid in equimolecular proportions at atmospheric temperature, the reaction being substantially instantaneous. Suitable organic acids are monocarboxylic fatty acids of 8 to about 22 carbon atoms, monohydric mononuclear phenols, and monocarboxylic petroleum naphthenic acids of about 8 to about 29 carbon atoms. These mono-acid salts offer the advantage of increased fuel oil solubility over the corresponding polyamine, especially with the lower members of the series, e.g., ethylene diamine and diethylene triamine. They are particularly desirable for the preparation of concentrated solutions in normally liquid hydrocarbons.

Representative monocarboxylic fatty acids of this invention are oleic acid, caprylic acid, pelargonic (nonanoic) acid, undecylic acid, lauric acid, stearic acid, linoleic acid, linolinic acid, behenic acid, and the like. Oleic acid is preferred.

Representative monohydric mononuclear phenols are phenol, the cresols, the ethyl phenols, the xylenols, and the like. Particularly desirable are the commercially available mixtures known as "cresylic acids" (a mixture of o-, m- and p-cresols) and "xylenols." Such mixtures result in mixtures of the mono-acid polyamine salts of the several phenols. The cresylic acid salts or cresylates of the examples were prepared from such "cresylic acids" and hence are mixtures of the mono-acid salts of the several cresols in said "cresylic acids."

The monocarboxylic petroleum naphthenic acids have the formula  $RCO_2H$ , wherein R is a naphthenic radical. The naphthenic radicals are predominantly those from cyclopentane, its homologs and bicyclic derivatives. The carboxyl group is usually attached to a paraffinic side chain of the ring, but may be directly attached to a ring carbon atom. The commercially available products, obtained from various petroleum sources, are mixtures of naphthenic acids of from 7 or 8 to about 29 carbon atoms, usually not more than 20 carbon atoms and averaging about 12 to 14 carbon atoms, sometimes also containing minor proportions of fatty acids and carboxylic acids derived from cyclohexane and its homologs. Refined commercial naphthenic acids generally have an apparent molecular weight of about 200-250 which corresponds to an average of 12 to 14 carbon atoms in the molecule. The naphthenic acid mono salts or mono-naphthenates of the examples were prepared from such

refined commercial naphthenic acids, and hence are mixtures of the mon-acid salts of the several naphthenic acids.

Representative mono-acid salts of this invention which have been found to be particularly satisfactory for the purposes of this invention are:

Ethylene diamine monooleate  
1,2-propylene diamine monooleate  
2,3-butylene diamine monooleate  
Diethylene triamine monooleate  
Ethylene diamine mononaphthenate  
Diethylene triamine mononaphthenate  
Ethylene diamine monocresylate  
Diethylene triamine monocresylate

15 The hydrocarbon distillate fuel oils, to which the polyamino compounds of this invention are to be added, are the hydrocarbon distillates which are heavier than gasoline and which are known to the art as furnace oil, burner oil, heating oil, range oil, diesel fuel, jet fuel, and fuel oil. In general, these oils have a boiling range of from about 300° F. to about 750° F. Also, the hydrocarbon distillate fuel oils contain active mercaptans. Active mercaptans are those which, when fuel oil containing them is brought into contact with copper, copper compounds or brass, will react therewith to form copper mercaptides that form copper mercaptide gels. The most active mercaptans are the aliphatic mercaptans, the activity thereof decreasing from the primary to the secondary to the tertiary mercaptans. Usually, aromatic mercaptans alone do not form solid copper mercaptide gels but, in the presence of an aliphatic primary mercaptan, they and the aliphatic secondary and tertiary mercaptans appear to contribute to the formation 30 of such gels.

35 The occurrence of mercaptans of all types in distillate hydrocarbon fuel oils is well known. Commercial hydrocarbon distillate fuel oils offered today for heating use, contain, when fresh from as low as 0.001% to as high as 0.03% by weight of mercaptan sulfur. This mercaptan sulfur content varies, depending on the source of the fuel oil, its processing history, and its age. For example, the mercaptan sulfur content of catalytic cracked fuel oil tends to diminish on aging, which may 40 be attributed to the reaction of mercaptans with olefin groups under conditions of storage. Thus, while the tendency of some fuel oils to form sludge increases on aging, the tendency to form copper mercaptide gel may actually decrease during this same period. Even quite 45 minute quantities of active mercaptan sulfur in a fuel oil tends to result in objectionable troublesome fouling of equipment, that is, small quantities of active mercaptan sulfur cause the deposition of rather large volumes of fuel oil as an insoluble gelatinous precipitate.

50 Generally, the quantity of polyamino compound of this invention which will be added to a hydrocarbon distillate fuel oil is from 0.1 to about 5 parts by weight for each part of active mercaptan sulfur present in the fuel oil, preferably from about 0.5 to about 3 parts by weight. For most hydrocarbon distillate fuel oils, this 55 will be from 0.0001% to about 0.15% by weight based on the fuel oil, preferably from about 0.0005% to about 0.1%. Larger amounts of polyamino compound may be used, but generally will be wasteful unless the fuel oil contains unusually large amounts of active mercaptan sulfur or it is to be used in equipment which is already fouled with copper mercaptide gel.

60 A polyamino compound of this invention or a mixture of any two or more thereof may be added as such to the hydrocarbon distillate fuel oil at atmospheric temperature or, if desired, at moderately elevated temperature and stirring until solution is complete. Preferably, the polyamino compound or mixture of compounds will be added in the form of a concentrated solution 65 in a normally liquid hydrocarbon, such as benzene,

toluene, xylene, gasoline, kerosene, fuel oils, and the like. Generally, the polyamino compounds will be in a concentration of from about 15% to about 70% by weight, preferably from about 30% to about 50% by weight. These concentrated solutions represent the commercial form in which the polyamino compound will be shipped to the refiner for addition to the fuel oil to be treated. Such solutions are more convenient to transport, to handle (e.g. pour) and to measure. The maximum concentration obtainable will depend upon the solubility of the polyamino compound in the liquid hydrocarbon and, for this purpose, it will be most desirable to employ those compounds of high solubility, preferably the mono-acid salts of the polyamines. Also, since the viscosity of the solution increases with increase in concentration of polyamino compound therein, the concentration generally will be limited by the maximum viscosity which can be efficiently poured and measured, usually a concentration of not more than about 50% by weight being optimum for this purpose.

For the purpose of breaking up and removing gel which has been formed in a system, an excess of polyamino compound may be incorporated in the fuel oil supply itself. However, this procedure will be fairly slow in removing the gel due to the low concentrations of the polyamino compound once it has finally diffused through the oil into the gel. On the other hand, rapid and effective breaking up of the gel has been obtained by adding the polyamino compound, as such, directly to the gel. However, it is preferred to employ concentrated solutions of the polyamino compound or of a mixture thereof in a normally liquid hydrocarbon. The concentrated solutions, described in the next preceding paragraph, are suitable for this purpose, preferably those in which the polyamino compounds are in a concentration of from about 15% to about 30% by weight, particularly in kerosene. As little as 1 part of polyamino compound is effective to liquefy up to 100 parts by weight of gel. Larger amounts may be used, but large excesses are wasteful.

In breaking up and removing gel from equipment which has become coated or fouled with the gel, it is desirable to bring the polyamino compounds rapidly into intimate contact with the gel, preferably by stirring the solution while it is in contact with the equipment. If the part of the equipment which carries the gelatinous deposit is readily removable (e.g. a filter screen), it can be immersed in a solution of the polyamino compound until the gel is completely broken up and then rinsed in a normally liquid hydrocarbon, such as kerosene, xylene, gasoline, or fuel oil, which is free of polyamino compound. If a domestic oil burner becomes plugged with gel during operation with an untreated fuel oil, the polyamino compound can be added to the system at any point which leads to the affected parts. For example, the feed lines can be disconnected from the fuel oil storage tank, and the fuel remaining therein drained or blown out and replaced by a concentrated solution of the polyamino compound. The system is then tested for normal flow. The cleaning operation can be repeated as may be necessary, using fresh solution or recirculating the old solution through the contaminated parts, e.g., nozzle, filter screen, or feed line. Finally, the equipment should be rinsed with a normally liquid hydrocarbon which does not contain polyamino compound, as before. Since concentrated solutions of the polyamino compounds are rather corrosive to copper in the presence of oxygen and/or moisture, it is desirable to wash such solutions from copper surfaces as soon as possible after the polyamino compounds have broken up the gels, i.e., to rinse them as set forth above.

The particular polyamino compound or mixture thereof employed will depend upon the manner and form in which it is to be used and the results desired, i.e., whether

it is to be used or handled in a concentrated solution, the concentration thereof, and whether it is to be used to break up preformed gel. While any of the polyamino compounds of this invention may be used very effectively to inhibit copper mercaptide gel formation in fuel oil, it will be preferred to employ any one or more of ethylene diamine, diethylene trimine, the propylene diamines, the dipropylene triamines, and the monoleates and mono-naphthenates of those polyamines. In breaking up or liquefying preformed copper mercaptide gel, the polyamino compounds vary in effectiveness, hexamethylene diamine being much less effective for this purpose than those diamines in which the amino groups are separated by fewer carbon atoms, the effectiveness increasing with decrease in the number of carbon atoms separating the amino groups. Thus, in breaking up preformed gel, it is preferred to employ alkylene diamines in which the two amino groups are separated by 2 to 4 carbon atoms, especially 2 to 3 carbon atoms, and dialkylene triamines in which each amino group is separated from the nearest other amino group by 2 to 3 carbon atoms.

Higher polyalkylene polyamines, i.e., the trialkylene tetramines and the tetraalkylene pentamines, have little or no effect to inhibit the formation of copper mercaptide gel in fuel oil or to break up preformed gel. For example, it has been found that tetraethylene pentamine neither inhibits nor breaks up copper mercaptide gel. Similarly, when the polyamines of this invention are alkylated to convert one or both of the primary amino groups to a secondary or a tertiary amino group, such as the N-alkyl, N-N-dialkyl, or N,N'-dialkyl-substituted compounds, their effectiveness for the purposes of this invention is greatly decreased or destroyed.

The polyamino compounds of this invention may be employed in hydrocarbon distillate fuel oils along with other additives which are conventionally employed to impart other desirable characteristics to the base oil, such as resistance to discoloration and the formation of sludge and to improve the combustion of the oil.

In order to more clearly illustrate this invention, suitable modes of carrying it into effect, and the advantageous results to be obtained thereby, the following examples are given in which the polyamino compounds employed are technical grade products and the salts were prepared by mixing one mole of the organic acid, carboxylic acid or phenol, with one mole of the polyamine at room temperature:

*Example I*

50 A five ml. portion of catalytically cracked fuel oil containing (a) a total of 0.4 weight percent mercaptan sulfer present as added dodecyl mercaptan and (b) 0.1 weight percent of ethylene diamine was mixed with a five ml. portion of fuel oil containing 0.4 weight percent 55 copper present as added copper naphthenate. No insoluble gel formed; the mixture remaining mobile and free of gel indefinitely (for at least several weeks).

In a control experiment, under identical conditions except that no ethylene diamine was present, immediate 60 gelation of the fuel took place.

When ethylene diamine was replaced in the above example by an equal weight of any of the following polyamines, complete inhibition of solid gel formation was observed: 1, 2-propylene diamine, 1,3-propylene diamine, 1,3-butylene diamine, hexamethylene diamine, diethylene triamine, di-(1,3-propylene) triamine. The mixture, in each case, remained free of gel indefinitely.

In contrast, solid gel was formed immediately when 70 0.2 weight percent of tetraethylene pentamine was employed in Example 1 instead of 0.1 weight percent of the above polyamines of this invention. Solid gel formed in 10 minutes when as much as 2 weight percent of 3-diethylaminopropylamine was similarly tested as an inhibitor; likewise, with 2 weight percent of 3-isopro-

pylaminopropylamine present the mixture solidified to gel in 30 minutes.

*Example 2*

A solid copper mercaptide gel was prepared by mixing (a) an equal volume of catalytically cracked fuel oil containing 0.4 weight percent mercaptan sulfur, present as added dodecyl mercaptan, with (b) an equal volume of fuel oil containing 0.4% copper, present as added copper naphthenate. To samples of this solid gel (9 parts each) was added from 0.15 to 0.25 part of diethylene triamine and the mixture was shaken. In a few moments, the gel broke up (completely liquefied), in each case, the original straw color changing to the bluish-green color of the copper-polyamine complex.

*Example 3*

Solid copper mercaptide gel (containing 0.2 weight percent copper) was prepared by mixing equal volumes of catalytically cracked fuel oil containing, respectively, 0.4 weight percent mercaptan sulfur as a 1:1 mixture of dodecyl and xylyl mercaptans and 0.4% copper as the naphthenate. One part samples of the gel were broken-up by adding 0.1 part of oleic acid mono salt of ethylene diamine (prepared by mixing 1 mole of oleic acid and 1 mole of ethylene diamine).

Substantially the same results, i.e. complete break up of the gel, are obtained on replacing the above ethylene diamine monooleic acid salt with any of the following polyamino compounds of this invention:

Cresylic acid mono salt of ethylene diamine (0.2 part)  
Naphthenic acid mono salt of ethylene diamine (0.2 part)  
Naphthenic acid mono salt of diethylene triamine (0.4 part)  
Oleic acid mono salt of diethylene triamine (0.6 part of a 33 1/3 weight percent solution in xylene i.e. 0.2 part active ingredient)  
Oleic acid mono salt of 1,2-propylene diamine (0.6 part of a 50 weight percent solution in xylene containing 0.3 part active ingredient)  
Oleic acid mono salt of 2,3-butylene diamine (0.4 part)

*Example 4*

An accelerated test, simulating field conditions, was devised to determine the sensitivity of fuel oils to copper mercaptide gel formation and to evaluate the effectiveness of various materials as inhibitors of gel formation. The test comprises passing or circulating (i.e. any number of passes) a sample of fuel oil over a specially prepared (corroded) copper strip, at a specified temperature and rate of flow, and then determining the increase in weight of the copper strip as a measure of the quantity of gel produced in a given time.

The corroded copper strips are specially prepared to speed up gel formation and to provide uniform conditions for the test. Preparation of corroded copper for the copper mercaptide gel test is as follows:

Copper strips, approximately 0.25 inch x 2.5 inches, are roughly polished with 00 emery cloth, steel wool-polished until uniformly bright, then washed with light naphtha, and dried in air. The copper strips may be stored in a tightly capped bottle for 10-15 days. 150 ml. of benzene and 30 ml. of concentrated aqueous ammonium hydroxide are mixed and shaken vigorously for 2 to 3 minutes to saturate the benzene with ammonia. The mixture is allowed to separate for 15 to 20 minutes and the aqueous layer is drawn off and discarded. Two or three polished copper strips, prepared as described above, are immersed in the ammonia-saturated benzene for 24 hours. The resulting corroded copper strips are dried by allowing the benzene to evaporate in air and then stored in a tightly capped bottle until needed.

When fuel oil which is normally subject to copper mercaptide gel formation in the field, i.e. contains naturally

occurring active mercaptans, is allowed to flow over a corroded copper strip (prepared as above described) at a rate of one liter per 24 hours at 37° F., a characteristic yellowish gelatinous deposit is present on the copper strip after 24 hours. Fuel oils giving a negative test, i.e. no gel appears and the copper strip shows no gain in weight, are considered free of active mercaptans, i.e. those forming insoluble copper mercaptide gel.

In order to determine under controlled conditions the effectiveness of various materials in preventing insoluble gel, the active mercaptan content of fuel oil samples were standardized by incorporating in them known quantities of active mercaptans such as dodecyl mercaptan or 1:1 mixture of dodecyl mercaptan and xylyl mercaptan.

In the following test, catalytically cracked fuel oil, containing (a) a total of 0.005 weight percent of active mercaptan sulfur (approximately 0.04 g. S/liter), which was added to the fuel oil as 1:1 dodecyl and xylyl mercaptans, and (b) 0.0006 weight percent of diethylene triamine monooleate, was passed over a pre-weighed corroded copper strip (prepared as described above) at a rate of 1 liter/24 hours at 37° F. At the end of 24 hours, the copper strip was washed with cyclohexane, air-dried and weighed. There was no increase in the weight of the copper strip.

In a control experiment under identical conditions and using the same base fuel containing the above mercaptans but with no added inhibitor present, the increase in weight of the copper strip was 0.1462 g.

Following the above-described test procedure, any of the polyamines of this invention may be employed to inhibit the formation of gelatinous deposit on copper; the copper strip remains clean and shows essentially no increase in weight.

It will be understood that the examples are given for illustrative purposes solely and that this invention is not limited to the specific embodiments disclosed therein. While only certain polyamino compounds and compositions have been employed in the examples, mixtures of any two or more thereof may be similarly employed. Also, other polyamino compounds and compositions, within the general disclosure, may be substituted therefor. Furthermore, the proportions, conditions, procedures, etc. may be varied widely as pointed out in the general description, without departing from the spirit and scope of this invention.

From the preceding disclosure, it is apparent that this invention provides novel means and methods for inhibiting the formation of copper mercaptide gels in hydrocarbon distillate fuel oils and for liquefying gels already formed and removing them from equipment coated or fouled therewith. It provides fuel oil compositions which are stabilized against the formation of such gels and concentrated solutions useful for preparing such fuel oil compositions and for breaking up preformed gels and cleaning equipment containing them. Thus, this invention solves serious problems of the art and constitutes a valuable improvement in and contribution to the art.

The embodiments of the invention in which an exclusive property or privilege is claimed are defined as follows:

1. A hydrocarbon distillate fuel oil which is in contact with a member of the group consisting of copper, copper compounds and brass, and which contains at least one mercaptan which normally tends to form a copper mercaptide gel, and a small proportion sufficient to inhibit such gel formation of at least one polyamino compound of the group consisting of alkylene primary diamines of 2 to 10 carbon atoms in which the primary amino groups are separated by 2 to 6 carbon atoms, dialkylenetriamines of 4 to 10 carbon atoms in which the amino groups are separated by 2 to 4 carbon atoms and two of the amino groups are primary amino groups, and mono-acid salts of said diamines and said triamines in which the acids are selected from the group consisting of monocarboxylic fatty acids of 8 to about 22 carbon atoms, monohydric mono-

nuclear phenols, and monocarboxylic petroleum naphthenic acids of about 8 to about 29 carbon atoms, said polyamino compound being in a proportion equivalent to 0.1 to about 5 parts of polyamino for each part of active mercaptan sulfur in the fuel oil.

2. A hydrocarbon distillate fuel oil which is in contact with a member of the group consisting of copper, copper compounds and brass, and which contains at least one mercaptan which normally tends to form a copper mercaptide gel, and from about 0.5 to about 3 parts by weight for each part of active mercaptan sulfur present in the fuel oil of at least one polyamino compound of the group consisting of alkylene primary diamines of 2 to 10 carbon atoms in which the primary amino groups are separated by 2 to 6 carbon atoms, dialkylene triamines of 4 to 10 carbon atoms in which the amino groups are separated by 2 to 4 carbon atoms and two of the amino groups are primary amino groups, and mono-acid salts of said diamines and said triamines in which the acids are selected from the group consisting of monocarboxylic fatty acids of 8 to about 22 carbon atoms, monohydric mononuclear phenols, and monocarboxylic petroleum naphthenic acids of about 8 to about 29 carbon atoms.

3. A hydrocarbon distillate fuel oil which is in contact with a member of the group consisting of copper, copper compounds and brass, and which contains at least one mercaptan which normally tends to form a copper mercaptide gel, and a small proportion sufficient to inhibit such gel formation of at least one alkylene primary diamine of 2 to 10 carbon atoms in which the primary amino groups are separated by 2 to 6 carbon atoms, said diamine being in a proportion of 0.1 to about 5 parts thereof for each part of active mercaptan sulfur in the fuel oil.

4. A hydrocarbon distillate fuel oil which is in contact with a member of the group consisting of copper, copper compounds and brass, and which contains at least one mercaptan which normally tends to form a copper mercaptide gel, and a small proportion sufficient to inhibit such gel formation of at least one alkylene primary diamine of 2 to 6 carbon atoms in which the primary amino groups are separated by 2 to 3 carbon atoms, said diamine being in a proportion of 0.1 to about 5 parts thereof for each part of active mercaptan sulfur in the fuel oil.

5. A hydrocarbon distillate fuel oil which is in contact with a member of the group consisting of copper, copper compounds and brass, and which contains at least one mercaptan which normally tends to form a copper mercaptide gel, and a small proportion sufficient to inhibit such gel formation of at least one propylene primary diamine in which the primary amino groups are separated by 2 to 3 carbon atoms, said diamine being in a proportion of 0.1 to about 5 parts thereof for each part of active mercaptan sulfur in the fuel oil.

6. A hydrocarbon distillate fuel oil which is in contact with a member of the group consisting of copper, copper compounds and brass, and which contains at least one mercaptan which normally tends to form a copper mercaptide gel, and a small proportion sufficient to inhibit such gel formation of at least one dialkylene triamine of 4 to 10 carbon atoms in which the amino groups are separated by 2 to 4 carbon atoms and two of the amino groups are primary amino groups, said triamine being in a proportion of 0.1 to about 5 parts thereof for each part of active mercaptan sulfur in the fuel oil.

7. A hydrocarbon distillate fuel oil which is in contact with a member of the group consisting of copper, copper compounds and brass, and which contains at least one mercaptan which normally tends to form a copper mercaptide gel, and a small proportion sufficient to inhibit such gel formation of at least one dialkylene triamine of 4 to 8 carbon atoms in which the amino groups are separated by 2 to 3 carbon atoms and two of the amino groups are primary amino groups, said triamine being in a proportion of 0.1 to about 5 parts thereof for each part of active mercaptan sulfur in the fuel oil.

8. A hydrocarbon distillate fuel oil which is in contact with a member of the group consisting of copper, copper compounds and brass, and which contains at least one mercaptan which normally tends to form a copper mercaptide gel, and a small proportion sufficient to inhibit such gel formation of diethylene triamine, said triamine being in a proportion of 0.1 to about 5 parts thereof for each part of active mercaptan sulfur in the fuel oil.

9. A hydrocarbon distillate fuel oil which is in contact with a member of the group consisting of copper, copper compounds and brass, and which contains at least one mercaptan which normally tends to form a copper mercaptide gel, and a small proportion sufficient to inhibit such gel formation of at least one mono-acid salt of an alkylene primary diamine of 2 to 10 carbon atoms in which the primary amino groups are separated by 2 to 6 carbon atoms, the acid component of said salt being a monocarboxylic fatty acid of 8 to about 22 carbon atoms, said salt being in a proportion equivalent to 0.1 to about 5 parts of diamine for each part of active mercaptan sulfur in the fuel oil.

10. A hydrocarbon distillate fuel oil which is in contact with a member of the group consisting of copper, copper compounds and brass, and which contains at least one mercaptan which normally tends to form a copper mercaptide gel, and a small proportion sufficient to inhibit such gel formation of at least one monooleate of an alkylene primary diamine of 2 to 6 carbon atoms in which the primary amino groups are separated by 2 to 3 carbon atoms, said monooleate being in a proportion equivalent to 0.1 to about 5 parts of diamine for each part of active mercaptan sulfur in the fuel oil.

11. A hydrocarbon distillate fuel oil which is in contact with a member of the group consisting of copper, copper compounds and brass, and which contains at least one mercaptan which normally tends to form a copper mercaptide gel, and a small proportion sufficient to inhibit such gel formation of ethylene diamine monooleate, said monooleate being in a proportion equivalent to 0.1 to about 5 parts of ethylene diamine for each part of active mercaptan sulfur in the fuel oil.

12. A hydrocarbon distillate fuel oil which is in contact with a member of the group consisting of copper, copper compounds and brass, and which contains at least one mercaptan which normally tends to form a copper mercaptide gel, and a small proportion sufficient to inhibit such gel formation of at least one mono-acid salt of a dialkylene triamine of 4 to 10 carbon atoms in which the amino groups are separated by 2 to 4 carbon atoms and two of the amino groups are primary amino groups, the acid component of said salt being a monocarboxylic fatty acid of 8 to about 22 carbon atoms, said salt being in a proportion equivalent to 0.1 to about 5 parts of triamine for each part of active mercaptan sulfur in the fuel oil.

13. A hydrocarbon distillate fuel oil which is in contact with a member of the group consisting of copper, copper compounds and brass, and which contains at least one mercaptan which normally tends to form a copper mercaptide gel, and a small proportion sufficient to inhibit such gel formation of at least one monooleate of a dialkylene triamine of 4 to 8 carbon atoms in which the amino groups are separated by 2 to 3 carbon atoms and two of the amino groups are primary amino groups, said monooleate being in a proportion equivalent to 0.1 to about 5 parts of triamine for each part of active mercaptan sulfur in the fuel oil.

14. A hydrocarbon distillate fuel oil which is in contact with a member of the group consisting of copper, copper compounds and brass, and which contains at least one mercaptan which normally tends to form a copper mercaptide gel, and a small proportion sufficient to inhibit such gel formation of diethylene triamine monooleate, said monooleate being in a proportion equivalent to 0.1 to about 5 parts of diethylene triamine for each part of active mercaptan sulfur in the fuel oil.

15. A composition for liquefying a gel, formed by the action of a copper mercaptide on a normally liquid hydrocarbon, which composition consists essentially of a normally liquid hydrocarbon having dissolved therein, in a concentration of from about 15% to about 70% by weight, at least one polyamino compound of the group consisting of alkylene primary diamines of 2 to 10 carbon atoms in which the primary amino groups are separated by 2 to 6 carbon atoms, dialkylenetriamines of 4 to 10 carbon atoms in which the amino groups are separated by 2 to 4 carbon atoms and two of the amino groups are primary amino groups, and mono-acid salts of said diamines and said triamines in which the acids are selected from the group consisting of monocarboxylic fatty acids of 8 to about 22 carbon atoms, monohydric mononuclear phenols, and monocarboxylic petroleum naphthenic acids of about 8 to about 29 carbon atoms.

16. A composition for liquefying a gel, formed by the action of a copper mercaptide on a normally liquid hydrocarbon, which composition consists essentially of a normally liquid hydrocarbon having dissolved therein, in a concentration of from about 15% to about 50% by weight, at least one mono-acid salt of an alkylene primary diamine of 2 to 10 carbon atoms in which the primary amino groups are separated by 2 to 6 carbon atoms, the acid component of said salt being a monocarboxylic fatty acid of 8 to about 22 carbon atoms.

17. A composition for liquefying a gel, formed by the action of a copper mercaptide on a normally liquid hydrocarbon, which composition consists essentially of a normally liquid hydrocarbon having dissolved therein, in a concentration of from about 15% to about 50% by weight, at least one mono-acid salt of a dialkylenetriamine of 4 to 10 carbon atoms in which the amino groups are separated by 2 to 4 carbon atoms and two of the amino groups are primary amino groups, the acid component of said salt being a monocarboxylic fatty acid of 8 to about 22 carbon atoms.

18. The process for liquefying a gel, formed by the action of a copper mercaptide on a normally liquid hydrocarbon, which comprises adding to said gel at least 1% by weight of at least one polyamino compound of the group consisting of alkylene primary diamines of 2 to 10

carbon atoms in which the primary amino groups are separated by 2 to 6 carbon atoms, dialkylenetriamines of 4 to 10 carbon atoms in which the amino groups are separated by 2 to 4 carbon atoms and two of the amino groups are primary amino groups, and mono-acid salts of said diamines and said triamines in which the acids are selected from the group consisting of monocarboxylic fatty acids of 8 to about 22 carbon atoms, monohydric mononuclear phenols, and monocarboxylic petroleum naphthenic acids of about 8 to about 29 carbon atoms.

19. The process for liquefying a gel, formed by the action of a copper mercaptide on a normally liquid hydrocarbon, which comprises adding to said gel at least 1% by weight of at least one alkylene primary diamine of 2 to 4 carbon atoms in which the primary amino groups are separated by 2 to 3 carbon atoms.

20. A hydrocarbon distillate fuel oil which is in contact with a member of the group consisting of copper, copper compounds and brass, and which contains at least one mercaptan which normally tends to form a copper mercaptide gel, and a small proportion sufficient to inhibit such gel formation of 1,2-propylene diamine monooleate, said monooleate being in a proportion equivalent to 0.1 to about 5 parts of the diamine for each part of active mercaptan sulfur in the fuel oil.

#### References Cited in the file of this patent

#### UNITED STATES PATENTS

|    |           |                |                |
|----|-----------|----------------|----------------|
| 30 | 2,204,234 | Schulze        | June 11, 1940  |
|    | 2,329,251 | Chenicek       | Sept. 14, 1943 |
|    | 2,369,490 | Proell         | Feb. 13, 1945  |
|    | 2,503,627 | McBride et al. | Apr. 11, 1950  |
|    | 2,559,574 | Weissberg      | July 3, 1951   |
| 35 | 2,759,875 | Bowers         | Aug. 21, 1956  |
|    | 2,851,344 | Marsh et al.   | Sept. 9, 1958  |

#### OTHER REFERENCES

"Organic Nitrogen Compounds," Carbide and Carbon Chem. Corp., rec'd March 27, 1950, page 4.

40 "Industrial Solvents," by Mellan, Second Ed., 1950, Reinhold Pub. Corp., N.Y., page 424.

"How's Your Fuel-Oil Quality?" Osterhout et al., Petroleum Processing, January 1956, pages 67-71.

UNITED STATES PATENT OFFICE  
CERTIFICATE OF CORRECTION

Patent No. 2,980,518

April 18, 1961

Philip L. Bartlett

It is hereby certified that error appears in the above numbered patent requiring correction and that the said Letters Patent should read as corrected below:

Column 2, line 40, for "brough" read -- brought --; column 3, line 51, for "mixturese" read -- mixtures --; column 4, line 2, for "mon-acid" read -- mono-acid --; column 6, line 7, for "trimine" read -- triamine --; line 8, for "monoleates" read -- monooleates --; column 9, line 4, for "polyamino" read -- polyamine --; column 10, line 16, for "prmiary" read -- primary --; column 11, line 34, for "whcih" read -- which --.

Signed and sealed this 10th day of October 1961.

(SEAL)

Attest:

ERNEST W. SWIDER

Attesting Officer

DAVID L. LADD

Commissioner of Patents

USCOMM-DC